

# UNITED STATES PATENT OFFICE.

GEORGE O. SEWARD AND FRANZ VON KÜGELGEN, OF HOLCOMBS ROCK, VIRGINIA, ASSIGNEES  
TO VIRGINIA LABORATORY COMPANY, OF NEW YORK, N. Y., A CORPORATION OF NEW  
YORK.

## PRODUCTION OF BARIUM AND BARIUM ALLOYS.

No. 900,962.

Specification of Letters Patent.

Patented Oct. 13, 1908.

Application filed March 28, 1906. Serial No. 308,577.

*To all whom it may concern:*

Be it known that we, GEORGE O. SEWARD, a citizen of the United States, and FRANZ VON KÜGELGEN, a subject of the German Emperor, both residing at Holcombs Rock, in the county of Bedford and State of Virginia, have jointly invented certain new and useful Improvements in the Production of Barium and Barium Alloys, of which the following is a specification.

This invention relates to the production of barium or alloys thereof by the electrolysis of a barium salt or compound.

Barium has been produced by electrolyzing barium chlorid, using a cathode of mercury, and obtaining a mercury-barium alloy from which the mercury is separated by distillation. This process is not practical, and does not produce barium in a pure state. Efforts have been made to produce barium by electrolyzing molten barium chlorid with an iron cathode, but without success, the barium separating in so fine a state of division that it would float to the anode, and there recombine with the halogen. The failure was probably due to the cathode not being small enough. We have found that by sufficiently decreasing the size of the cathode the metal is obtained in molten globules.

The present invention provides a method of producing barium in a molten state by using an iron cathode with a sufficiently high current density and a suitable electrolyte. If molten barium chlorid is used as the electrolyte, it is very difficult to keep its temperature low enough for practical results, and if the temperature is not kept at the right point, the separated metal has a tendency to redissolve in the electrolyte.

We have discovered that much better results are obtained if barium fluorid is added to the barium chlorid, which has the result of lowering the melting point of the electrolyte, and diminishing the tendency of the barium to redissolve therein.

If we wish to produce metallic barium, we

submit a molten mixture of barium chlorid and barium fluorid to electrolysis, with an iron cathode, maintaining the current at a sufficiently high density. If we wish to obtain alloys of barium, we use as the cathode the metal with which it is desired that the barium should alloy. The proportions of barium chlorid to the barium fluorid or other salt to be electrolyzed, may vary within wide limits; we have successfully used a mixture of 90 per cent. by weight of barium chlorid and 10 per cent. by weight of barium fluorid.

Instead of barium fluorid, any other barium salt may be substituted that will lower the melting point of the electrolyte and diminish the tendency of the barium to redissolve therein. Mixtures of barium salts may also be used.

We claim as our invention:—

1. The process which consists in electrolyzing fused barium chlorid with the addition of a barium salt of lower melting point.

2. The process which consists in electrolyzing fused barium chlorid with the addition of barium fluorid.

3. The process which consists in electrolyzing a barium salt with the addition of a barium salt of lower melting point, by means of a cathode of a metal capable of alloying with barium, whereby to produce an alloy of such metal with barium.

4. The process which consists in electrolyzing a fused mixture of barium chlorid and barium fluorid, by means of a cathode of a metal capable of alloying with barium, whereby to produce an alloy of such metal with barium.

In witness whereof, we have hereunto signed our names in the presence of two subscribing witnesses.

GEORGE O. SEWARD.  
FRANZ VON KÜGELGEN.

Witnesses:

F. V. TRIDDER,  
J. H. WEBB.